

Patented July 19, 1927.

1,636,491

UNITED STATES PATENT OFFICE.

DANIEL MANSON SUTHERLAND, JR., OF TRENTON, NEW JERSEY.

ELECTRIC INSULATION BOARD.

No Drawing.

Application filed November 11, 1924. Serial No. 749,345.

My invention has for its object the economical production of insulating boards, sheets, and bodies of varied form, having a cellulose base, possessing high dielectric properties and capable of being readily machined, and finished in any desired color or colors, or to simulate natural woods, stones and the like.

Better to differentiate the present invention from the known prior art it may be stated that under existing practice, electrical insulation products having a cellulose base are prepared by making what is known as hard or vulcanized fiber, zinc chloride, or sulphuric and nitric acids being used to dissolve the cellulose.

Products thus made are laminated, and absorb water or moisture somewhat freely, for which reasons they are unsuitable for use where high dielectric or insulating effect is sought.

The prior art discloses many combinations of binders with cellulose, designed to give, but not giving the results which I have successfully attained by my new formula and procedure. Prior plans have involved the use of cellulose with various binders, such as asphalt, resin, and oil soaps, and the product has in some cases been given a surface coating of cellulose acetate; but as heretofore supplied, such compositions have been found deficient in dielectric properties, absorbent of moisture, and difficult to drill or machine, to finish in the various ways deemed desirable, or to engrave.

For general uses, the material produced should be non-absorbent and devoid of tackiness, but highly dielectric, capable of being drilled, machined, engraved, or finished to present in color and surface an appearance substantially identical with those producible with or upon wood, stone and other substances, natural or artificial, and, finally, these qualities should be stable and lasting.

Procedure under the present invention consists in combining cellulose and a suitable binder or binders to produce a pulp, forming the pulp into a sheet, board, block or other body, drying the same, coating it with a suitable film, compressing or compacting it under heat and pressure, and finally cooling it while still under pressure.

This process produces what is commonly known as the homogeneous board, and this is the preferred form of the product. I can, however, produce on a cylinder wet machine,

sheets, with laminations, which are, however, so closely compacted or so firmly compressed by pressure and heat, followed by cooling under pressure, that such sheets closely resemble in quality the homogeneous product.

For sheets or boards up to  $\frac{1}{4}$  inch in thickness I prefer to use the cylinder wet machine; but for thicknesses greater than  $\frac{1}{4}$  inch I prefer to use a hydraulic wet machine such as set forth in Letters Patent of the United States granted to me March 4, 1924, and numbered 1,485,894.

The relative proportions of cellulose and binder are highly important, and in great measure determine the qualities or characteristics of the finished product. Thus a high percentage or proportion of cellulose, say 70% by weight of the composition or mixture, gives a product which does not drill cleanly or smoothly, has a high water absorption, and presents a surface strongly resembling enamel, or patent leather, whereas a less glossy but smooth and even surface is generally deemed desirable. Materially lower percentage of cellulose, say 40% or thereabout, gives much better results.

Again, I have found that the resultant product is better when special care is taken to incorporate the binder with the cellulose in finely divided condition, the fibers being in such case more certainly and completely surrounded or encompassed by the binder or binders.

The best composition and procedure that I have thus far developed through careful experimentation and practical use will now be stated, it being understood however, that reasonable variation in proportions and substitutions of equivalents can be made without materially or greatly affecting the result.

A composition is formed comprising cellulose, and a binder, preferably consisting of china wood oil soap or linseed oil soap, or a mixture of the two, together with gilsonite. The following formula has given very satisfactory results:

|               | Per cent. | 105 |
|---------------|-----------|-----|
| Cellulose     | 40        |     |
| Oil soap      | 15        |     |
| Acaroid resin | 2         |     |
| Gilsonite     | 43        |     |
|               |           | 110 |
|               | 100       |     |

The oil soaps are prepared by cooking,

either in an open or in a closed vessel, china wood oil, or linseed oil with caustic soda, until complete saponification is effected. The acaroid resin is dissolved in caustic soda and mixed with the oil soap or soaps in the proportion above stated.

The gilsonite is ground in water until it is so fine that about 95% will pass through a 100 mesh screen, and after screening is 10 mixed with the oil soap or soaps. The binder so prepared is then intimately mixed with the cellulose, and alum is used in quantity sufficient to neutralize the caustic soda and to precipitate the soap or soaps and acaroid 15 resin in insoluble form upon the cellulose fibers. The gilsonite is in this manner held in suspension with the fibers, thus avoiding its subsequent loss during formation of the sheet, board or other body.

20 The use of oil soaps and acaroid resin alone does not produce the desired results, since in the absence of gilsonite the product, after compression or compaction, will gradually swell when the pressure is withdrawn, 25 thus lessening its density and its water-resisting properties.

Gilsonite is employed in preference to other and similar agents because it melts under the temperature and pressure which obtains 30 during compression or compaction, and when subsequently cooled while the mass is still under pressure, it firmly cements together the cellulose fibers, and thus prevents in great degree the reswelling of the formed 35 sheet or body when the pressure is discontinued. The surface of the formed body also remains smooth for a longer period of time in consequence of the presence and action of the gilsonite.

40 The use of oil soap improves the sanding or surfacing qualities of the finished body, and overcomes the tendency of gilsonite to gum abrasives, or to glaze and render ineffective abrading and polishing wheels and 45 surfaces.

The acaroid resin plays an important part in improving water resistance or rendering the product non-absorbent by causing the oil soaps to precipitate in a finely divided 50 state, which would not happen in the absence of the acaroid resin.

A surface coating or film is applied to the article after it is formed and dried, in order to prevent the binders from adhering to the 55 contacting surfaces of the hot press, dies, or moulds in which the material is compressed and fashioned, and for the further purpose of affording or permitting a high polish.

I prefer for the surface film or coating, 60 cellulose acetate or cellulose nitrate lacquers, which may be applied by dipping, spraying, or brushing. These lacquers can be colored before application by the use of suitable aniline dyes, soluble in alcohol, and may be applied in solid color, or to simulate different 65

woods, stones and other natural substances or materials.

When the composition is adequately compressed and compacted to produce a density of not less than 300 grains per cubic inch, 70 and is cooled while still under pressure, an insulating material is produced which has high dielectric properties, good machining qualities, and a smooth and even surface, and which is non-absorbent or water repellent. 75

It will be seen from the foregoing description that I have produced a nicely balanced composition of matter, in which each ingredient has and performs its own special and important office and function, combining, co-operating, or reacting with or upon other ingredients in a manner to produce, under the described procedure, a highly efficient 80 insulating material, of excellent appearance, and capable of being fashioned and finished 85 without difficulty, and of being made to simulate very closely more expensive natural substances.

As above indicated, I have given the best formula known to me, but am aware that 90 reasonable latitude is possible in the selection of ingredients possessing similar properties, and in the proportions of different ingredients employed. It is hence to be understood that I do not mean to limit myself to 95 the use of the precise ingredients named, or to the exact proportions stated; but may vary each within reasonable limits. Thus, by way of example, a single oil soap or a plurality of such soaps may be used, the aggregate quantity being in each instance substantially that above proposed. So too, cellulose acetate or cellulose nitrate may be employed, cellulose acetate producing in some respects a better article than cellulose nitrate, but cellulose nitrate being somewhat 100 economical.

The process or method of manufacture can be carried out with ordinary apparatus, requiring no special description because common and well known to those engaged in the manufacture of paper pulp and pulp products. 110

In an application filed in my name on the 4th day of August, 1924, Serial No. 730,022, I 115 have set forth the use of acaroid resin in a film or coating applied to the surface of insulating sheets, boards and forms having a cellulose base, such film or coating serving to prevent adhesion of the insulating body 120 when subjected to heat and pressure, or subsequent to such compression under heat. Under the present plan, however, acaroid resin is incorporated in or is an ingredient 125 of the binder, and is hence thoroughly commingled with the pulp mass; whereas under the prior application it was present only in the surface film or coating and not distributed throughout the mass. This application is accordingly designed to claim and cover 130

specifically such incorporation of the acaroid resin in the pulp mass.

By requirement of the Patent Office this application is in its claims restricted to the 5 composition, the method or process of forming, shaping, finishing, and imparting stability to the product or products made from the composition herein set forth being carried into a divisional application, Serial No. 10 85,582, filed February 2, 1926.

What is claimed is:—

1. An electric insulation composition comprising cellulose, oil soap, acaroid resin, and gilsonite in substantially the stated proportions, by weight.

2. A material for electrical insulation con-

sisting of the following ingredients in substantially the stated proportions, by weight, that is to say: cellulose 40%, oil soap 15%, acaroid resin 2% and gilsonite 43%, the gilsonite being distributed throughout the mass and coating the individual fibers of the cellulose. 20

3. A compressed and compacted insulating body consisting of the following ingredients 25 in substantially the proportions of: cellulose 40%, oil soap 15%, acaroid resin 2%, and gilsonite 43%, by weight.

In testimony whereof I have signed my name to this specification.

DANIEL MANSON SUTHERLAND, Jr.